

J. R. POWELL & B. G. CASLER,  
ROOFING AND SIDING MATERIAL,  
APPLICATION FILED APR. 30, 1913.

1,114,032.

Patented Oct. 20, 1914.

FIG. 1.



FIG. 2.



FIG. 3.



FIG. 6.



Inventors

Witnesses

Edwin L. Bradford  
M. D. Ballauf

John R. Powell  
Benjamin G. Casler  
By  
Ritter & Fitter

Attorneys

# UNITED STATES PATENT OFFICE.

JOHN R. POWELL, OF WAUKEGAN, ILLINOIS, AND BENJAMIN G. CASLER, OF TONAWANDA, NEW YORK.

## ROOFING AND SIDING MATERIAL.

1,114,032.

Specification of Letters Patent.

Patented Oct. 20, 1914.

Application filed April 30, 1913. Serial No. 764,577.

To all whom it may concern:

Be it known that we, JOHN R. POWELL and BENJAMIN G. CASLER, citizens of the United States, residing at Waukegan, in the county of Lake and State of Illinois, and at Tonawanda, in the county of Erie and State of New York, respectively, have invented certain new and useful Improvements in Roofing and Siding Material; and we do hereby declare the following to be a full, clear, and exact description of the invention, such as will enable others skilled in the art to which it appertains to make and use the same.

Our invention relates to the production of that class of manufactures, commonly termed "construction material," wherein one or more plies of roofing-felt or similar material is saturated with a waterproof substance and coated with asphalt or its equivalent to render it waterproof, and then surfaced with mica, slate, sand, gravel or like heat resisting material to produce a building fabric having a fire resisting wearing surface. This class of building material has heretofore been produced in several ways, for example, by development on the roof or in like position where applied, and also in the form of finished articles of trade, as for instance, in the form of surfaced roofing and siding sheets, shingles, tiles and the like individual articles.

Our present invention relates especially to this latter form of construction material, that is to say, the finished article of trade, and more particularly to that class wherein the heat and wear-resisting surfaced portions of the fabric or construction material are so related as to simulate a shingled or tessellated structure or surface. Heretofore this particular class of construction material has possessed either the ultimate fractional form or the unit of design, as for instance, having the appearance and dimensions of a shingle or tile, or the extended character, such as sheet or integer, the surface of which is made up of a multiple of the units of design.

In the production of the shingle, tile, or like unit or fractional form of the construction material, a previously prepared strip saturated and having an adhesive or bed coating of asphaltum and a layer covering of grit or its equivalent heat and wear-resisting surface, is severed into shingle or tile units, if shingle or tile units are de-

sired, or is severed at intervals by kerfing, if the strip is to simply simulate shingles, and when so produced the trade article is unwarrantedly expensive in the manufacture and marketing thereof, lacks durability in service by reason of the severed edge exposure of the fabric, absorption of moisture, and the curling of the edges under the action of the heat and sun's rays. Moreover, in the case of the kerfed strip the construction material is greatly weakened and undergoes rapid deterioration.

In the production of the sheet form or integer of multiple units, the method of production practised has been to apply to the saturated and asphaltum coated sheet a uniform or continuous layer or covering of grit or equivalent heat and wear resisting surfacing, and to apply to portions of said grit or heat and wear resisting surface a superposed coating of asphaltum in such forms or outlines as to produce contrasts which simulate the units of the structure it is desired to imitate, whether the same be shingle or tile. This form of the trade article not only renders its production unnecessarily expensive, but renders the article less desirable in that the sheet does not possess uniform strength throughout, and is pitted, which permits the accumulation of water at intervals on the fabric, thus hastening its deterioration.

The object, therefore, of our present invention is the production of a trade article, to wit, a construction material strip of uniform strength, increased weather and wear-resisting properties, and having characteristics which adapt it ready to architectural ornamentation, and which can be produced at a minimum cost for labor and material.

To this end our invention, generally stated, consists in a roofing fabric strip having the portion intended to be exposed to the weather protected by an exposed embedded grit layer distributed in spaced tessellæ alternating with uncovered contrasting portions.

There are other, minor, features of invention, all as will hereinafter more fully appear.

In the drawing chosen for the purpose of illustrating our invention, the scope whereof is pointed out in the claims, Figure 1 illustrates the construction material strip in the preferred form, that is to say, of double

width to better adapt it for reeling and covering for shipment. Fig. 2 illustrates the single width strip in one of the forms in which it may be advantageously utilized either as roofing or siding. Fig. 3 illustrates one method of applying the construction strips, as such, to a structure, in utilizing the same either as roofing or as siding. Fig. 4 is a detail transverse section, taken on the line 4—4, Fig. 1; Fig. 5 is a view corresponding to Fig. 4, but illustrating a modification of our invention. Fig. 6 illustrates a grid or stop-out sheet of the configuration used in surfacing the construction material shown in Figs. 1, 2 and 3 of the drawing.

Like symbols refer to like parts wherever they occur.

We will now proceed to describe our invention more fully so that others skilled in the art to which it appertains may apply the same.

A strip of roofing felt of suitable width to accommodate the design or configuration of the surfaced portion A plus the width of the unsurfaced or lap portion B adjacent thereto is required, as indicated in Fig. 2 of the drawing, but for purposes of convenience in manufacturing and shipping, a strip of twice said width, as shown in Fig. 1 of the drawing, is preferably selected. This strip of roofing felt, either single or double width as the case may be, is saturated with suitable waterproofing material and coated with asphalt as in the manner now practised in the manufacture of ready roofing fabrics. In applying the coating of asphalt or like substance, and previous to the application of the surfacing material, strands of wire or flat metal 1 may if desired be embedded at intervals in the asphalt coating. As the strip of felt or other foundation material comes from the asphalt bath or coating machine it may be, and preferably is, led under a scraper which is so adjusted with reference to the non-surfaced portion B of the strip as to remove therefrom all or any desired part of the asphalt coating. As will hereinafter appear the scraper is preferably arranged so as to cause the asphalt coating to taper or diminish in thickness from the surfaced portion A of the sheet toward the line a which corresponds to the margin adjacent to the unsurfaced or lap portion of the individual strips into which the sheet of double width illustrated in Fig. 1 is designed to be divided. While the coating of asphalt on the fabric is in the proper condition to receive the surfacing material of mica, sand, gravel or the like, the strip is covered, at one margin in case of a single width strip or at both margins in case of a double width strip, by a grid or stopout sheet C which corresponds in form to the pattern of surface material desired at the margin or margins of the strip. While so covered the

strip passes beneath the grit hopper which deposits the surfacing material on the uncovered portions of the surface of the strip. From the grid or stop out, or when the grid or stop out has been removed the strip passes to rolls which press the surfacing material into the coated marginal surface or surfaces of the fabric, causing the displaced coating material of asphalt to extrude and fill up the intervals between the surfacing material thus obtaining a substantially level weather surface, the embedded grit causing the extruded or displaced coating material to pass into the unsurfaced intervals thus insuring the uniform strength of the fabric throughout.

The design of the grid is not material and, therefore, it may be of any desired pattern or configuration which will preserve unsurfaced division lines between the units of the design being provided for.

In the present instance the marginal figure chosen for purposes of illustrating our invention is one of rectangular form, as indicated at 2, or rather a series of such rectangular forms arranged at regular intervals along the margin or margins of the strip and separated from each other by narrow spaces 3, to thus simulate the bricks in a wall or the exposed portions of overlapping shingles.

The strips are to be utilized in strip form for either roofing or siding, the surfaced design and the non-surfaced intermediate portions 3 of the coated fabric permit the designs of adjacent strips to be arranged to break joints and thus simulate either shingles for roofing purposes, or bricks or blocks for siding purposes.

As shown in Fig. 4, it is preferred to cup or incline the unsurfaced central portion of the double width strip of felt or foundation 4 to thus cause the individual strips into which the double strip is separated along the longitudinal line a to have tapering lap edges or lap margins 5. When foundation material thus tapered is employed, the surface of such tapering portion is preferably scraped substantially free of the asphalt coating in the course of manufacture while the asphalt coating is preferably gradually increased in thickness, as at 6, until it is of the desired thickness to retain the surfacing material 2. In this form of construction the wires or stiffeners 1, which are embedded in the asphalt coating, preferably terminate, as shown, at the beginning of the tapering portion 5 of the felt or foundation material.

In the modified form of construction illustrated in Fig. 5, in which the felt or foundation sheet is of uniform thickness throughout, the stiffening wires 1<sup>a</sup>, 1<sup>b</sup>, which are embedded in the asphalt coating, extend to or substantially to the center of the sheet, the asphalt being tapered or diminished in

thickness, as at 7, 7, from the surfacing material 2 in opposite directions toward the division line *a* of the double width sheet. When the double sheet is separated along the 5 central line *a* each of the individual strips thus formed has an unsurfaced, tapered, marginal portion 7, as will be readily understood. The tapering of the felt and asphalt not only effects an economy in these 10 materials, but results in affording a better contact between the overlapping portions of the strips as well as in eliminating any sharp turns or bends incident to the covering of one strip with another.

15 In case a double width strip as shown in Fig. 1 of the drawing is produced, which, as before noted, is the preferred form, a slight cut at mid-width and longitudinally of the strip is made, as indicated at *a*. Such cut, 20 while of sufficient depth to insure the easy separation of the fabric by force, should not be sufficiently deep to permit accidental separation of the strips during the normal operations of rolling and covering the strips for 25 shipment.

In order to prevent the adherence of the fabric if the same is to be formed into a roll for shipment, either of several well known plans may be adopted. For instance, the 30 non-surfaced margin of the strip may be dusted or it may be covered with tissue paper as is now commonly done for a like purpose.

When utilized in strip form, as is preferred, the strips may be applied lengthwise 35 or vertically of the structure covered thereby (from peak to eaves in roofing), and may be secured in the usual way by nails and cement, thus facilitating and cheapening the cost of application to buildings.

40 In preparing for shipment, as an article

of trade, the strips may be rolled and covered as in the case of ready roofing sheets, and the labor and cost of crating and boxing required for shipment of articles such a shingles, etc., may thus be avoided in construction material embodying our invention. 45

Furthermore, there is a material saving of asphalt and grit or surfacing material in the manufacture of the article in strip form rather than in the unit form of shingles, 50 tiles, or the like.

We claim:

1. As an article of manufacture, a roofing fabric strip comprised of an asphalt coated fabric having the portion intended to be exposed to the weather protected at intervals by exposed embedded grit distributed in spaced tessellæ alternating with the exposed asphalt coated surface of the fabric. 55

2. As an article of manufacture a roofing fabric strip comprised of an asphalt coated fabric having the portion intended to be exposed to the weather protected at intervals by exposed embedded grit distributed in spaced tessellæ alternating with narrow exposed portions of the coated surface of the fabric. 60 65

In testimony whereof we affix our signatures, in presence of two subscribing witnesses.

JOHN R. POWELL.  
BENJAMIN G. CASLER.

Witnesses as to the signature of John R. Powell:

C. T. HEYDUKER,  
ROY J. MASON.

Witnesses as to the signature of Benjamin G. Casler:

SPINER B. PERKIN,  
MARGARET MAHONEY.